



US012366069B2

(12) **United States Patent**  
**Boss et al.**

(10) **Patent No.:** US 12,366,069 B2  
(45) **Date of Patent:** Jul. 22, 2025

(54) **ROOFING MATERIALS WITH SYNTHETIC ROOFING GRANULES AND METHODS OF MAKING THEREOF**

(71) Applicant: **BMIC LLC**, Dallas, TX (US)

(72) Inventors: **Daniel E. Boss**, Morris Township, NJ (US); **Ming-Liang Shiao**, Basking Ridge, NJ (US); **Luis Duque**, Hackensack, NJ (US)

(73) Assignee: **BMIC LLC**, Dallas, TX (US)

(\*) Notice: Subject to any disclaimer, the term of this patent is extended or adjusted under 35 U.S.C. 154(b) by 0 days.

(21) Appl. No.: **18/746,209**

(22) Filed: **Jun. 18, 2024**

(65) **Prior Publication Data**

US 2024/0337103 A1 Oct. 10, 2024

**Related U.S. Application Data**

(63) Continuation of application No. 18/311,583, filed on May 3, 2023, now Pat. No. 12,044,011, which is a continuation of application No. 17/696,007, filed on Mar. 16, 2022, now Pat. No. 11,680,409.

(60) Provisional application No. 63/161,483, filed on Mar. 16, 2021.

(51) **Int. Cl.**

**E04D 1/20** (2006.01)  
**E04D 1/00** (2006.01)  
**E04D 1/26** (2006.01)

(52) **U.S. Cl.**  
CPC ..... **E04D 1/20** (2013.01); **E04D 2001/005** (2013.01); **E04D 1/26** (2013.01)

(58) **Field of Classification Search**  
CPC ..... E04D 1/20; E04D 1/26; E04D 2001/005  
See application file for complete search history.

(56) **References Cited**

**U.S. PATENT DOCUMENTS**

|                 |         |                   |
|-----------------|---------|-------------------|
| 7,354,596 B1    | 4/2008  | Banovetz et al.   |
| 8,673,427 B2    | 3/2014  | Kalkanoglu et al. |
| 8,997,427 B2    | 4/2015  | Kalkanoglu et al. |
| 9,057,194 B2    | 6/2015  | Jenkins et al.    |
| 9,074,373 B2    | 7/2015  | Stahl             |
| 9,404,259 B2    | 8/2016  | Heulings et al.   |
| 9,538,762 B2    | 1/2017  | Bryson et al.     |
| 11,414,342 B2   | 8/2022  | Budd et al.       |
| 2002/0155770 A1 | 10/2002 | Van Niekerk       |
| 2005/0072114 A1 | 4/2005  | Shiao et al.      |
| 2007/0148342 A1 | 6/2007  | Kalkanoglu et al. |
| 2013/0095293 A1 | 4/2013  | Boss et al.       |
| 2013/0202852 A1 | 8/2013  | Shiao et al.      |
| 2014/0349072 A1 | 11/2014 | Hong et al.       |
| 2019/0185681 A1 | 6/2019  | Anderson et al.   |
| 2019/0300449 A1 | 10/2019 | Panzarella et al. |

*Primary Examiner* — Adriana Figueroa

(74) *Attorney, Agent, or Firm* — Venable LLP

(57) **ABSTRACT**

This invention, in embodiments, relates to a roofing material comprising (a) a coated substrate having a top surface and a back surface, and (b) a plurality of roofing granules applied to the top surface of the coated substrate. The plurality of roofing granules comprises from 50% to 100% of unitary, uncoated, non-mineral based particles. This invention, in embodiments, further relates to a method of preparing such roofing material.

**30 Claims, 5 Drawing Sheets**





| Type                   | Color          | CIELAB Color Space |       |      |      | Avg. Total Solar Reflectance |
|------------------------|----------------|--------------------|-------|------|------|------------------------------|
|                        |                | L*                 | a*    | b*   | E*   |                              |
| Mineral-Based Granules | Gray Green     | 44.6               | -2.6  | 3.0  | 44.8 | 0.2                          |
|                        | Green          | 32.3               | -13.4 | 9.9  | 36.3 | 0.1                          |
|                        | Red            | 30.3               | 18.2  | 15.6 | 38.7 | 0.1                          |
|                        | Dark Black     | 17.2               | 0.2   | 0.4  | 17.2 | 0.1                          |
|                        | Light Black    | 27.2               | -0.4  | -0.2 | 27.2 | 0.1                          |
|                        | Black          | 29.9               | -0.6  | -0.3 | 29.9 | 0.1                          |
|                        | Cinnamon       | 35.3               | 15.8  | 18.8 | 43.0 | 0.2                          |
|                        | Brown          | 23.2               | 6.2   | 5.7  | 24.6 | 0.1                          |
|                        | Desert Tan     | 46.4               | 6.5   | 11.2 | 48.2 | 0.2                          |
|                        | Buff           | 56.5               | 8.6   | 21.3 | 61.0 | 0.3                          |
|                        | White          | 76.9               | -0.1  | 2.1  | 77.0 | 0.5                          |
|                        | Off-White      | 61.5               | -0.1  | 0.7  | 61.5 | 0.3                          |
|                        | Gray           | 48.0               | -1.0  | -1.9 | 48.1 | 0.2                          |
| Synthetic Granules     | Black n Grain  | 17.2               | 0.1   | 0.1  | 17.2 | 0.1                          |
|                        | Charcoal Gray  | 32.9               | 0.4   | 1.1  | 32.9 | 0.2                          |
|                        | Cool Gray      | 31.9               | -0.6  | -2.8 | 32.0 | 0.3                          |
|                        | Dark Bronze    | 28.9               | 0.1   | -0.9 | 28.9 | 0.2                          |
|                        | Dark Brown     | 30.3               | 1.0   | 1.0  | 30.3 | 0.2                          |
|                        | Dark Grey      | 26.7               | 1.2   | 1.2  | 26.8 | 0.2                          |
|                        | Desert Tan     | 35.2               | 2.0   | 2.9  | 35.4 | 0.3                          |
|                        | Energy Tan     | 43.4               | 3.8   | 12.3 | 45.3 | 0.4                          |
|                        | Goldenrod      | 53.1               | 9.8   | 30.0 | 61.7 | 0.5                          |
|                        | Hartford Green | 47.7               | 6.9   | 27.4 | 55.4 | 0.2                          |
|                        | Ivy Green      | 43.1               | 1.1   | 16.6 | 46.2 | 0.2                          |
|                        | Patina Green   | 35.8               | -7.9  | 3.3  | 36.8 | 0.2                          |
|                        | Regal Blue     | 34.8               | -5.4  | 1.3  | 35.2 | 0.2                          |
|                        | Regal Red      | 33.9               | 6.7   | 6.9  | 35.2 | 0.3                          |
|                        | RV Almond      | 51.0               | 10.3  | 9.9  | 53.0 | 0.7                          |
|                        | RV Beige       | 51.7               | 11.5  | 15.7 | 55.3 | 0.2                          |
|                        | RV Gray        | 62.5               | 0.2   | 8.9  | 63.2 | 0.5                          |
|                        | Smoke Gray     | 50.1               | -0.8  | -1.3 | 50.1 | 0.3                          |
|                        | Terra Cotta    | 38.6               | 4.3   | 3.3  | 38.9 | 0.3                          |
|                        | White 299      | 95.0               | -0.7  | 3.9  | 95.1 | 0.8                          |

**FIG. 2**



*FIG. 3*

| Sample | Granule Type      | Color          | Particle Shape | Particle Geometry (LxWxH) (in.) | CIELab Color Space |      |      | Avg. Total Solar Reflectance (%) | Shingle Wt./Thickness/Area (g/mil/in <sup>2</sup> ) |
|--------|-------------------|----------------|----------------|---------------------------------|--------------------|------|------|----------------------------------|-----------------------------------------------------|
|        |                   |                |                |                                 | L*                 | a*   | b*   |                                  |                                                     |
| 1      | Mineral-Based     | Gray Green     | Cubical        | 0.04x0.04x0.04                  | 44.1               | -3.5 | 2.2  | 44.3                             | 12.2%                                               |
| 2      | Mineral-Based     | Brown          | Cubical        | 0.06x0.06x0.06                  | 24.3               | 6.1  | 7.5  | 26.2                             | 4.7%                                                |
| 3      | Mineral-Based     | White          | Cubical        | 0.05x0.05x0.06                  | 64.7               | -1.2 | 0.6  | 64.7                             | 31.8%                                               |
| 4      | Non Mineral-Based | Hartford Green | Rod            | 0.13x0.07                       | 35.3               | -8.3 | -5.7 | 36.7                             | 18.8%                                               |
| 5      | Non Mineral-Based | Dark Brown     | Rod            | 0.13x0.06                       | 23.5               | 3.1  | 3.6  | 24.0                             | 16.6%                                               |
| 6      | Non Mineral-Based | White 299      | Spherical      | 0.1x0.1                         | 85.6               | -0.6 | 2.3  | 85.6                             | 64.7%                                               |

FIG. 4

| Sample      | Granule Type      | Color   | CIELab Color Measurement |      |      | Staining Index ( $\Delta E^*$ ) |
|-------------|-------------------|---------|--------------------------|------|------|---------------------------------|
|             |                   |         | L*                       | a*   | b*   |                                 |
| 1 (initial) | Mineral-Based     | I-760   | 49.7                     | -2.4 | -1.5 | 3.3                             |
| 1 (after)   |                   |         | 47.3                     | -1.6 | 0.6  |                                 |
| 2 (initial) | Non Mineral-Based | RV Grey | 60.8                     | -4.7 | -1.3 | 0.4                             |
| 2 (after)   |                   |         | 60.5                     | -4.6 | -1.2 |                                 |

**FIG. 5****FIG. 6**

## ROOFING MATERIALS WITH SYNTHETIC ROOFING GRANULES AND METHODS OF MAKING THEREOF

### RELATED APPLICATION

This application is a continuation of U.S. patent application Ser. No. 18/311,583, filed May 3, 2023, which is a continuation of U.S. patent application Ser. No. 17/696,007, filed Mar. 16, 2022, now U.S. Pat. No. 11,680,409, which claims the priority of U.S. provisional application Ser. No. U.S. 63/161,483, entitled "Roofing Materials With Synthetic Roofing Granules And Methods of Making Thereof" filed Mar. 16, 2021, which are incorporated herein by reference in their entirety for all purposes.

### FIELD OF THE INVENTION

This invention relates to roofing materials having synthetic roofing granules and methods of making these roofing materials. By preparing roofing materials such as, e.g., shingles, using synthetic or non-mineral based roofing granules, these roofing materials can exhibit superior properties of, for example, reduced weight, improved or higher solar reflectance, reduced staining, improved color saturation and/or gloss, as compared to roofing materials having traditional, mineral-based roofing granules.

### BACKGROUND OF THE INVENTION

Traditional roofing materials, such as, e.g., shingles, are based upon a glass or felt mat that is coated and impregnated with an asphalt-based composition that is coated with granules. These granules, which are typically mineral-based particles, are applied to the surface of the shingles to protect the shingle, while also providing additional coloring and/or textures to thus, enhance the aesthetics of the shingle. Generally, the mineral-based particles are mined from rock that is dense, which results in a significant increase in the weight of the shingle. Additionally, the mineral-based particles are typically dark in color for the necessary UV opacity to protect the asphaltic materials of the shingle from degradation over time, while also having a rough surface as a result of crushing the material to size. As a result, these dark-color, rough granules have a tendency to absorb high levels of solar radiation, while the rough surfaces decrease reflectivity of the granules. This absorption of high levels of solar radiation, as well as the decreased reflectivity of the granules can result in a "hot roof," which can lead to an increase in the cooling energy needed to keep the indoor air comfortable during summer seasons.

As discussed above, roofing granules comprising mineral-based particles can significantly increase the weight of the shingle, such that the shingles become heavy to handle and/or the design of multiple layers of shingles is limited due to the heavy weight of the final shingle product. Also, the mineral-based roofing granules have a tendency to absorb oils from the asphalt of the shingles, which results in an undesirable "stained" or "darkened" color of the shingle.

There is thus a need for synthetic or non-mineral based roofing granules for preparing roofing materials that exhibit reduced weight, improved solar reflectance, reduced staining, improved color and/or gloss, as compared to roofing materials having traditional, mineral-based roofing granules.

### SUMMARY OF THE INVENTION

One embodiment of this invention pertains to a roofing material comprising (a) a coated substrate having a top

surface and a back surface, and (b) a plurality of roofing granules applied to the top surface of the coated substrate. The plurality of roofing granules comprises from 50% to 100% of unitary, uncoated, non-mineral based particles.

5 In one embodiment, the substrate comprises one of a fiberglass mat, a polyester mat, a scrim, a coated scrim, or a combination thereof.

In one embodiment, the roofing material is one of a roofing shingle and a roofing tile.

10 In one embodiment, the roofing material is one of (i) an asphaltic shingle, (ii) a non-asphaltic shingle, and (ii) a polymer-modified asphalt shingle.

In some embodiments, each roofing granule of the plurality of roofing granules has a density of 1.2 g/cm<sup>3</sup> to 2.5 g/cm<sup>3</sup>.

15 In one embodiment, the non-mineral based particles comprise a synthetic particle.

In one embodiment, the non-mineral based particles comprise at least one of a thermoplastic polymer, filled polymers, filled rubbers, filled plastics, a polymer-sand composite, a rubber particle, a recycled material, a wood filled polymer, a bio-based particle, a thermoset material, a fiber-reinforced polymer, and combinations thereof.

20 25 In one embodiment, the non-mineral based particles have an aspect ratio of from 1.5 to 50. In another embodiment, the non-mineral based particles have an aspect ratio of from 5 to 30.

In one embodiment, the non-mineral based particles have 30 a particle size of #8 US mesh to #60 US mesh.

In one embodiment, less than 1% by weight of the plurality of roofing granules have a particle size of greater than #100 US mesh.

35 In an embodiment, the roofing material exhibits a lower weight per thickness as compared to a roofing material prepared with roofing granules comprising a majority of mineral based particles.

In one embodiment, the roofing material exhibits a weight 40 per thickness of 1 to 3 g/mil<sup>2</sup>.

In one embodiment, the roofing material exhibits an improved staining resistance as compared to a roofing material prepared with roofing granules comprising a majority of mineral based particles.

45 In an embodiment, the roofing granules exhibit a total solar reflectance (TSR) of 0.2 to 0.8 according to ASTM C1549.

In one embodiment, the roofing granules exhibit a higher 50 color saturation as compared to roofing granules comprising mineral based particles.

Another embodiment of this invention pertains to a method of preparing a roofing material. The method includes (a) obtaining a coated substrate, (b) obtaining a plurality of roofing granules, wherein the plurality of roofing granules 55 comprises from 50% to 100% of unitary, uncoated, non-mineral based particles, and (c) applying the plurality of roofing granules to a surface of the coated substrate to form a roofing material.

In one embodiment, the step of applying the plurality of 60 roofing granules to the surface of the coated substrate is conducted to achieve an average surface coverage amount of the roofing granules of greater than 80%.

In one embodiment, the substrate comprises one of a fiberglass mat, a polyester mat, a scrim, a coated scrim, or 65 a combination thereof.

In some embodiments, the roofing material is one of a roofing shingle and a roofing tile.

In some embodiments, each roofing granule of the plurality of roofing granules has a density of 1.2 g/cm<sup>3</sup> to 2.5 g/cm<sup>3</sup>.

In one embodiment, the non-mineral based particles comprise a synthetic particle.

In one embodiment, the non-mineral based particles comprise at least one of a thermoplastic polymer, filled polymers, filled rubbers, filled plastics, a polymer-sand composite, a rubber particle, a recycled material, a wood filled polymer, a bio-based particle, a thermoset material, a fiber-reinforced polymer, and combinations thereof.

#### BRIEF DESCRIPTION OF THE FIGURES

For a more complete understanding of the invention and the advantages thereof, reference is made to the following descriptions, taken in conjunction with the accompanying figures, in which:

FIG. 1 is an illustration of a roofing material comprising synthetic or non-mineral based roofing granules according to an embodiment of the invention.

FIG. 2 is a table illustrating color space values and TSR values of mineral-based roofing granules as compared to synthetic or non-mineral based roofing granules according to embodiments of the invention.

FIG. 3 is a photograph of three different granule colors for both mineral-based roofing granules and non-mineral based roofing granules according to embodiments of the invention.

FIG. 4 is a table illustrating color space values, TSR values, and other measurements of mineral-based roofing granules as compared to synthetic or non-mineral based roofing granules according to embodiments of the invention.

FIG. 5 is a table illustrating color values and staining index values ( $\Delta E^*$ ) of mineral-based roofing granules as compared to synthetic or non-mineral based roofing granules according to embodiments of the invention.

FIG. 6 is a photograph illustrating the staining resistance of shingle samples prepared with mineral-based roofing granules as compared to synthetic or non-mineral based roofing granules according to embodiments of the invention.

#### DETAILED DESCRIPTION OF THE INVENTION

Among those benefits and improvements that have been disclosed, other objects and advantages of this disclosure will become apparent from the following description taken in conjunction with the accompanying figures. Detailed embodiments of the present disclosure are disclosed herein; however, it is to be understood that the disclosed embodiments are merely illustrative of the disclosure that may be embodied in various forms. In addition, each of the examples given regarding the various embodiments of the disclosure are intended to be illustrative, and not restrictive.

Throughout the specification and claims, the following terms take the meanings explicitly associated herein, unless the context clearly dictates otherwise. The phrases "in one embodiment," "in an embodiment," and "in some embodiments" as used herein do not necessarily refer to the same embodiment(s), though they may. Furthermore, the phrases "in another embodiment" and "in some other embodiments" as used herein do not necessarily refer to a different embodiment, although they may. All embodiments of the disclosure are intended to be combinable without departing from the scope or spirit of the disclosure.

As used herein, the term "based on" is not exclusive and allows for being based on additional factors not described,

unless the context clearly dictates otherwise. In addition, throughout the specification, the meaning of "a," "an," and "the" include plural references. The meaning of "in" includes "in" and "on."

As used herein, terms such as "comprising," "including," and "having" do not limit the scope of a specific claim to the materials or steps recited by the claim.

As used herein, terms such as "consisting of" and "composed of" limit the scope of a specific claim to the materials and steps recited by the claim.

All prior patents, publications, and test methods referenced herein are incorporated by reference in their entireties.

As used herein, the term "coated substrate" means a substrate that is coated on one side (upper surface or lower surface) or both sides (upper surface and lower surface) with a coating that includes, for example, an asphaltic coating, a non-asphaltic coating, and/or a polymer-modified asphalt coating. According to one embodiment, the "coated substrate" can also include a modified bitumen roll(s), a roll(s) of non-asphaltic roofing, metal shingles and/or tiles, and any other roofing tiles or elements where a granulated surface is desired.

As used herein, the term "weight percent" or "% by weight" means the percentage by weight of the roofing granules based upon a total weight of the roofing granules applied to the roofing material.

As used herein, the term "a majority of" means greater than 50% by weight.

As used herein, the term "roofing material" includes, but is not limited to, shingles, waterproofing membranes, underlayment, and tiles.

One embodiment of this invention pertains to a roofing material comprising (a) a coated substrate having a top surface and a back surface, and (b) a plurality of roofing granules applied to the top surface of the coated substrate. The plurality of roofing granules comprises from 50% to 100% of unitary, uncoated, non-mineral based particles.

FIG. 1 illustrates a roofing material (e.g., shingle) 100 according to an embodiment of the invention. In this embodiment, the roofing material 100 includes a coated substrate 110 having a front or top surface 112 and a back surface 115. The roofing material 100 further includes an upper portion or headlap portion 119 and a lower portion or buttlap portion 120. The buttlap portion 120 includes a series of cut-outs 114 leaving a plurality of tabs 116. The edge 113 of the buttlap portion 120 will be the lowermost or bottom edge of the roofing material 100 when installed onto a roof. Attached and/or laminated to the back surface 115 of the roofing material 100 is a backer strip 118. As shown in FIG. 1, the upper surface of the backer strip 118 is visible between the tabs 116 of the buttlap portion 120 of the coated substrate 110 of the roofing material 100.

The roofing material 100 of the embodiment of FIG. 1 further includes a plurality of roofing granules 150 disposed on the top surface 112 of the headlap portion 119, the plurality of tabs 116, and the backer strip 118. In an embodiment, the plurality of roofing granules comprises from 50% to 100% of unitary, uncoated, non-mineral based particles. In an embodiment, the plurality of roofing granules comprises from 60% to 100% of unitary, uncoated, non-mineral based particles. In an embodiment, the plurality of roofing granules comprises from 70% to 100% of unitary, uncoated, non-mineral based particles. In an embodiment, the plurality of roofing granules comprises from 75% to 100% of unitary, uncoated, non-mineral based particles. In an embodiment, the plurality of roofing granules comprises from 80% to 100% of unitary, uncoated, non-mineral based

particles. In an embodiment, the plurality of roofing granules comprises from 85% to 100% of unitary, uncoated, non-mineral based particles. In an embodiment, the plurality of roofing granules comprises from 90% to 100% of unitary, uncoated, non-mineral based particles. In an embodiment, the plurality of roofing granules comprises from 95% to 100% of unitary, uncoated, non-mineral based particles. In an embodiment, the plurality of roofing granules comprises from 50% to 90% of unitary, uncoated, non-mineral based particles. In an embodiment, the plurality of roofing granules comprises from 60% to 90% of unitary, uncoated, non-mineral based particles. In an embodiment, the plurality of roofing granules comprises from 70% to 90% of unitary, uncoated, non-mineral based particles. In an embodiment, the plurality of roofing granules comprises from 80% to 90% of unitary, uncoated, non-mineral based particles. In an embodiment, the plurality of roofing granules comprises from 50% to 80% of unitary, uncoated, non-mineral based particles. In an embodiment, the plurality of roofing granules comprises from 60% to 80% of unitary, uncoated, non-mineral based particles. In an embodiment, the plurality of roofing granules comprises from 70% to 80% of unitary, uncoated, non-mineral based particles. In an embodiment, the plurality of roofing granules comprises from 50% to 70% of unitary, uncoated, non-mineral based particles. In an embodiment, the plurality of roofing granules comprises from 60% to 70% of unitary, uncoated, non-mineral based particles. In an embodiment, the plurality of roofing granules comprises from 50% to 60% of unitary, uncoated, non-mineral based particles.

In an embodiment, the substrate (e.g., coated substrate 110) comprises one of a fiberglass mat, a polyester mat, a scrim, a coated scrim, or a combination thereof. In some embodiments, the substrate or mat includes nano-fibrillated cellulose fibers.

In an embodiment, the roofing material (e.g., roofing material 100) is one of a roofing shingle and a roofing tile. In some embodiments, the roofing material is one of (i) an asphaltic shingle, (ii) a non-asphaltic shingle, and (ii) a polymer-modified asphalt shingle. According to one embodiment, the roofing material is a roofing shingle that is one of (i) a single layer shingle or (ii) a laminated shingle having two or more layers.

In an embodiment, each roofing granule of the plurality of roofing granules has a density of 1 g/cm<sup>3</sup> to 3 g/cm<sup>3</sup>. In an embodiment, each roofing granule of the plurality of roofing granules has a density of 1.2 g/cm<sup>3</sup> to 3 g/cm<sup>3</sup>. In an embodiment, each roofing granule of the plurality of roofing granules has a density of 1.5 g/cm<sup>3</sup> to 3 g/cm<sup>3</sup>. In an embodiment, each roofing granule of the plurality of roofing granules has a density of 1.6 g/cm<sup>3</sup> to 3 g/cm<sup>3</sup>. In an embodiment, each roofing granule of the plurality of roofing granules has a density of 1.8 g/cm<sup>3</sup> to 3 g/cm<sup>3</sup>. In an embodiment, each roofing granule of the plurality of roofing granules has a density of 2 g/cm<sup>3</sup> to 3 g/cm<sup>3</sup>. In an embodiment, each roofing granule of the plurality of roofing granules has a density of 2.2 g/cm<sup>3</sup> to 3 g/cm<sup>3</sup>. In an embodiment, each roofing granule of the plurality of roofing granules has a density of 2.5 g/cm<sup>3</sup> to 3 g/cm<sup>3</sup>. In an embodiment, each roofing granule of the plurality of roofing granules has a density of 2.8 g/cm<sup>3</sup> to 3 g/cm<sup>3</sup>. In an embodiment, each roofing granule of the plurality of roofing granules has a density of 1 g/cm<sup>3</sup> to 2.5 g/cm<sup>3</sup>. In an embodiment, each roofing granule of the plurality of roofing granules has a density of 1.2 g/cm<sup>3</sup> to 2.5 g/cm<sup>3</sup>. In an embodiment, each roofing granule of the plurality of roofing granules has a density of 1.5 g/cm<sup>3</sup> to 2.5 g/cm<sup>3</sup>. In an embodiment, each roofing granule of the plurality of roofing granules has a density of 1.8 g/cm<sup>3</sup> to 2.5 g/cm<sup>3</sup>. In an embodiment, each roofing granule of the plurality of roofing granules has a density of 2 g/cm<sup>3</sup> to 2.5 g/cm<sup>3</sup>. In an embodiment, each roofing granule of the plurality of roofing granules has a density of 2.2 g/cm<sup>3</sup> to 2.5 g/cm<sup>3</sup>. In an embodiment, each roofing granule of the plurality of roofing granules has a density of 2.5 g/cm<sup>3</sup> to 2.5 g/cm<sup>3</sup>. In an embodiment, each roofing granule of the plurality of roofing granules has a density of 1 g/cm<sup>3</sup> to 2 g/cm<sup>3</sup>. In an embodiment, each roofing granule of the plurality of roofing granules has a density of 1.2 g/cm<sup>3</sup> to 2 g/cm<sup>3</sup>. In an embodiment, each roofing granule of the plurality of roofing granules has a density of 1.5 g/cm<sup>3</sup> to 2 g/cm<sup>3</sup>. In an embodiment, each roofing granule of the plurality of roofing granules has a density of 1.8 g/cm<sup>3</sup> to 2 g/cm<sup>3</sup>. In an embodiment, each roofing granule of the plurality of roofing granules has a density of 2 g/cm<sup>3</sup> to 2 g/cm<sup>3</sup>. In an embodiment, each roofing granule of the plurality of roofing granules has a density of 2.2 g/cm<sup>3</sup> to 2 g/cm<sup>3</sup>. In an embodiment, each roofing granule of the plurality of roofing granules has a density of 2.5 g/cm<sup>3</sup> to 2 g/cm<sup>3</sup>. In an embodiment, each roofing granule of the plurality of roofing granules has a density of 1 g/cm<sup>3</sup> to 1.6 g/cm<sup>3</sup>. In an embodiment, each roofing granule of the plurality of roofing granules has a density of 1.2 g/cm<sup>3</sup> to 1.6 g/cm<sup>3</sup>. In an embodiment, each roofing granule of the plurality of roofing granules has a density of 1.5 g/cm<sup>3</sup> to 1.6 g/cm<sup>3</sup>.

25 In an embodiment, the non-mineral based particles comprise a synthetic particle. In some embodiments, the non-mineral based particles comprise at least one of a thermoplastic polymer, filled polymers, filled rubbers, filled plastics, highly filled polymer particles, composite particles 30 of non-mineral materials, such as a polymer-sand composite, a rubber particle, a recycled material, a wood filled polymer, a bio-based particle, a thermoset material, a fiber-reinforced polymer, and combinations thereof. According to one embodiment, the particles can be highly filled with mineral 35 fillers, including, e.g., sands, stone fines, granule fines, calcium carbonates, clays, fly ashes, and combinations thereof. According to an embodiment, the particles can be filled with mineral fillers by up to 75% by weight.

In an embodiment, the non-mineral based particles can 40 contain functional fillers to improve processability, impact resistance, fire resistance, UV resistance, UV blocking, oxidation resistance, color stability, algae resistance, and combinations thereof, as well as fillers able to remove and/or trap a targeted chemical compound (such as, e.g., NO<sub>x</sub>, CO<sub>2</sub>, etc.). Also, according to an embodiment, the particles can have highly reflective pigments, such as, e.g., pigments comprising TiO<sub>2</sub>, metal oxides, graphene, perylene, transitional metal oxides, metallic pigments, pearlescent pigments, thin film coated pigments, solar reflective colorants, 45 solar reflective fillers, opacifiers, voids, or their combinations to increase the total solar reflectance of the particles.

50 According to an embodiment, the non-mineral based particles can be obtained via a number of processes, including, but not limited to, extrusion, co-extrusion, blending or mixing at elevated temperatures, or any agglomeration process to form the initial mass, followed by particle forming methods such as, e.g., crushing, impact-crushing, hammer mills, cryogenic crushing or grinding, roller mills, chopping or cutting after extrusion strand forming, injection molding, 55 compression molding, encapsulations, and combinations thereof.

According to an embodiment, the non-mineral based particles can have other structures such as, e.g., a core-shell structure to have different layers that can provide different 60 functionalities and/or to have a low-cost core covered with a durable, weatherable outer layer. Also, according to an embodiment, the non-mineral based particles can include a

biocide or algicide to help to control the roof algae growth and/or to maintain the aesthetics. Furthermore, according to an embodiment, the non-mineral based particles can have an adhesive promoter, a surface for promoting adhesion to asphalt, and/or a surface treated via plasma or flame or the like to promote its adhesion to an asphaltic coating.

According to an embodiment, the non-mineral based particles comprise one or more shapes, including, for example, round shapes, flat circles, squares, cylinders (including, e.g., flat cylinders, disk-shapes, rod shapes, and/or pancakes), flat rectangles (including, e.g., coasters), etc., and combinations thereof.

According to an embodiment, the non-mineral based particles have an aspect ratio, meaning a ratio between the smallest dimension to the largest dimension of the particles (e.g., a ratio of the thickness to the diameter of, for example, a disk-shaped particle and/or a ratio of the thickness to the length of, for example, a rod shaped particle), of from 1.5 to 50. According to another embodiment, the non-mineral based particles have an aspect ratio of from 2 to 50. According to an embodiment, the non-mineral based particles have an aspect ratio of from 3 to 50. According to an embodiment, the non-mineral based particles have an aspect ratio of from 5 to 50. According to an embodiment, the non-mineral based particles have an aspect ratio of from 10 to 50. According to an embodiment, the non-mineral based particles have an aspect ratio of from 15 to 50. According to an embodiment, the non-mineral based particles have an aspect ratio of from 20 to 50. According to an embodiment, the non-mineral based particles have an aspect ratio of from 25 to 50. According to an embodiment, the non-mineral based particles have an aspect ratio of from 30 to 50. According to an embodiment, the non-mineral based particles have an aspect ratio of from 40 to 50. According to an embodiment, the non-mineral based particles have an aspect ratio of from 1.5 to 40. According to an embodiment, the non-mineral based particles have an aspect ratio of from 2 to 40. According to an embodiment, the non-mineral based particles have an aspect ratio of from 3 to 40. According to an embodiment, the non-mineral based particles have an aspect ratio of from 5 to 40. According to an embodiment, the non-mineral based particles have an aspect ratio of from 10 to 40. According to an embodiment, the non-mineral based particles have an aspect ratio of from 15 to 40. According to an embodiment, the non-mineral based particles have an aspect ratio of from 20 to 40. According to an embodiment, the non-mineral based particles have an aspect ratio of from 25 to 40. According to an embodiment, the non-mineral based particles have an aspect ratio of from 30 to 40. According to an embodiment, the non-mineral based particles have an aspect ratio of from 1.5 to 30. According to an embodiment, the non-mineral based particles have an aspect ratio of from 2 to 30. According to an embodiment, the non-mineral based particles have an aspect ratio of from 3 to 30. According to an embodiment, the non-mineral based particles have an aspect ratio of from 5 to 30. According to an embodiment, the non-mineral based particles have an aspect ratio of from 10 to 30. According to an embodiment, the non-mineral based particles have an aspect ratio of from 15 to 30. According to an embodiment, the non-mineral based particles have an aspect ratio of from 20 to 30.

According to an embodiment, the non-mineral based particles have an aspect ratio of from 25 to 30. According to an embodiment, the non-mineral based particles have an aspect ratio of from 1.5 to 25. According to an embodiment, the non-mineral based particles have an aspect ratio of from 2 to 25. According to an embodiment, the non-mineral based

particles have an aspect ratio of from 3 to 25. According to an embodiment, the non-mineral based particles have an aspect ratio of from 5 to 25. According to an embodiment, the non-mineral based particles have an aspect ratio of from 10 to 25. According to an embodiment, the non-mineral based particles have an aspect ratio of from 15 to 25. According to an embodiment, the non-mineral based particles have an aspect ratio of from 20 to 25. According to an embodiment, the non-mineral based particles have an aspect ratio of from 1.5 to 20. According to an embodiment, the non-mineral based particles have an aspect ratio of from 2 to 20. According to an embodiment, the non-mineral based particles have an aspect ratio of from 3 to 20. According to an embodiment, the non-mineral based particles have an aspect ratio of from 5 to 20. According to an embodiment, the non-mineral based particles have an aspect ratio of from 10 to 20. According to an embodiment, the non-mineral based particles have an aspect ratio of from 15 to 20. According to an embodiment, the non-mineral based particles have an aspect ratio of from 1.5 to 15. According to an embodiment, the non-mineral based particles have an aspect ratio of from 2 to 15. According to an embodiment, the non-mineral based particles have an aspect ratio of from 3 to 15. According to an embodiment, the non-mineral based particles have an aspect ratio of from 5 to 15. According to an embodiment, the non-mineral based particles have an aspect ratio of from 10 to 15. According to an embodiment, the non-mineral based particles have an aspect ratio of from 1.5 to 10. According to an embodiment, the non-mineral based particles have an aspect ratio of from 2 to 10. According to an embodiment, the non-mineral based particles have an aspect ratio of from 3 to 10. According to an embodiment, the non-mineral based particles have an aspect ratio of from 5 to 10. According to an embodiment, the non-mineral based particles have an aspect ratio of from 1.5 to 5. According to an embodiment, the non-mineral based particles have an aspect ratio of from 2 to 5.

According to an embodiment, the non-mineral based particles have an aspect ratio of from 3 to 5. According to an embodiment, the non-mineral based particles have an aspect ratio of from 1.5 to 3. According to an embodiment, the non-mineral based particles have an aspect ratio of from 2 to 3. According to an embodiment, the non-mineral based particles have an aspect ratio of from 1.5 to 2. According to an embodiment, the non-mineral based particles have an aspect ratio of from 1 to 1.

In an embodiment, the non-mineral based particles have a particle size of #8 US mesh to #60 US mesh. In an embodiment, the non-mineral based particles have a particle size of #8 US mesh to #50 US mesh. In an embodiment, the non-mineral based particles have a particle size of #8 US mesh to #40 US mesh. In an embodiment, the non-mineral based particles have a particle size of #8 US mesh to #30 US mesh. In an embodiment, the non-mineral based particles have a particle size of #8 US mesh to #20 US mesh. In an embodiment, the non-mineral based particles have a particle size of #8 US mesh to #10 US mesh. In an embodiment, the non-mineral based particles have a particle size of #10 US mesh to #60 US mesh. In an embodiment, the non-mineral based particles have a particle size of #10 US mesh to #50 US mesh. In an embodiment, the non-mineral based particles have a particle size of #10 US mesh to #40 US mesh. In an embodiment, the non-mineral based particles have a particle size of #10 US mesh to #30 US mesh. In an embodiment, the non-mineral based particles have a particle size of #10 US mesh to #20 US mesh. In an embodiment, the non-mineral based particles have a particle size of #20 US

mesh to #60 US mesh. In an embodiment, the non-mineral based particles have a particle size of #20 US mesh to #50 US mesh. In an embodiment, the non-mineral based particles have a particle size of #20 US mesh to #40 US mesh. In an embodiment, the non-mineral based particles have a particle size of #20 US mesh to #30 US mesh. In an embodiment, the non-mineral based particles have a particle size of #30 US mesh to #60 US mesh. In an embodiment, the non-mineral based particles have a particle size of #30 US mesh to #50 US mesh. In an embodiment, the non-mineral based particles have a particle size of #30 US mesh to #40 US mesh. In an embodiment, the non-mineral based particles have a particle size of #40 US mesh to #60 US mesh. In an embodiment, the non-mineral based particles have a particle size of #40 US mesh to #50 US mesh. In an embodiment, the non-mineral based particles have a particle size of #50 US mesh to #60 US mesh.

In one embodiment, less than 50% by weight of the plurality of roofing granules have a particle size of greater than #100 US mesh. In an embodiment, less than 40% by weight of the plurality of roofing granules have a particle size of greater than #100 US mesh. In an embodiment, less than 30% by weight of the plurality of roofing granules have a particle size of greater than #100 US mesh. In an embodiment, less than 20% by weight of the plurality of roofing granules have a particle size of greater than #100 US mesh. In an embodiment, less than 10% by weight of the plurality of roofing granules have a particle size of greater than #100 US mesh. In an embodiment, less than 5% by weight of the plurality of roofing granules have a particle size of greater than #100 US mesh. In an embodiment, less than 1% by weight of the plurality of roofing granules have a particle size of greater than #100 US mesh.

In one embodiment, the roofing material exhibits a lower weight per thickness as compared to a roofing material prepared with roofing granules comprising a majority of mineral based particles.

In an embodiment, the roofing material exhibits a weight per thickness of 1 to 3 g/mil/ft<sup>2</sup>. In an embodiment, the roofing material exhibits a weight per thickness of 1.2 to 3 g/mil/ft<sup>2</sup>. In an embodiment, the roofing material exhibits a weight per thickness of 1.4 to 3 g/mil/ft<sup>2</sup>. In an embodiment, the roofing material exhibits a weight per thickness of 1.5 to 3 g/mil/ft<sup>2</sup>. In an embodiment, the roofing material exhibits a weight per thickness of 1.6 to 3 g/mil/ft<sup>2</sup>. In an embodiment, the roofing material exhibits a weight per thickness of 1.8 to 3 g/mil/ft<sup>2</sup>. In an embodiment, the roofing material exhibits a weight per thickness of 2 to 3 g/mil/ft<sup>2</sup>. In an embodiment, the roofing material exhibits a weight per thickness of 2.2 to 3 g/mil/ft<sup>2</sup>. In an embodiment, the roofing material exhibits a weight per thickness of 2.4 to 3 g/mil/ft<sup>2</sup>. In an embodiment, the roofing material exhibits a weight per thickness of 2.5 to 3 g/mil/ft<sup>2</sup>. In an embodiment, the roofing material exhibits a weight per thickness of 2.6 to 3 g/mil/ft<sup>2</sup>. In an embodiment, the roofing material exhibits a weight per thickness of 2.8 to 3 g/mil/ft<sup>2</sup>.

In an embodiment, the roofing material exhibits an improved staining resistance as compared to a roofing material prepared with roofing granules comprising a majority of mineral based particles.

In an embodiment, the roofing granules exhibit a total solar reflectance (TSR) of 0.2 to 0.8 according to ASTM C1549. In an embodiment, the roofing granules exhibit a total solar reflectance (TSR) of 0.3 to 0.8 according to ASTM C1549. In an embodiment, the roofing granules exhibit a total solar reflectance (TSR) of 0.4 to 0.8 according to ASTM C1549. In an embodiment, the roofing granules

exhibit a total solar reflectance (TSR) of 0.5 to 0.8 according to ASTM C1549. In an embodiment, the roofing granules exhibit a total solar reflectance (TSR) of 0.6 to 0.8 according to ASTM C1549. In an embodiment, the roofing granules exhibit a total solar reflectance (TSR) of 0.7 to 0.8 according to ASTM C1549. In an embodiment, the roofing granules exhibit a total solar reflectance (TSR) of 0.2 to 0.7 according to ASTM C1549. In an embodiment, the roofing granules exhibit a total solar reflectance (TSR) of 0.3 to 0.7 according to ASTM C1549. In an embodiment, the roofing granules exhibit a total solar reflectance (TSR) of 0.4 to 0.7 according to ASTM C1549. In an embodiment, the roofing granules exhibit a total solar reflectance (TSR) of 0.5 to 0.7 according to ASTM C1549. In an embodiment, the roofing granules exhibit a total solar reflectance (TSR) of 0.6 to 0.7 according to ASTM C1549. In an embodiment, the roofing granules exhibit a total solar reflectance (TSR) of 0.2 to 0.6 according to ASTM C1549. In an embodiment, the roofing granules exhibit a total solar reflectance (TSR) of 0.3 to 0.6 according to ASTM C1549. In an embodiment, the roofing granules exhibit a total solar reflectance (TSR) of 0.4 to 0.6 according to ASTM C1549. In an embodiment, the roofing granules exhibit a total solar reflectance (TSR) of 0.5 to 0.6 according to ASTM C1549. In an embodiment, the roofing granules exhibit a total solar reflectance (TSR) of 0.2 to 0.5 according to ASTM C1549. In an embodiment, the roofing granules exhibit a total solar reflectance (TSR) of 0.3 to 0.5 according to ASTM C1549. In an embodiment, the roofing granules exhibit a total solar reflectance (TSR) of 0.4 to 0.5 according to ASTM C1549. In an embodiment, the roofing granules exhibit a total solar reflectance (TSR) of 0.2 to 0.4 according to ASTM C1549. In an embodiment, the roofing granules exhibit a total solar reflectance (TSR) of 0.3 to 0.4 according to ASTM C1549. In an embodiment, the roofing granules exhibit a total solar reflectance (TSR) of 0.2 to 0.3 according to ASTM C1549.

In one embodiment, the roofing granules exhibit a higher color saturation as compared to roofing granules comprising mineral based particles.

Another embodiment of this invention pertains to a method of preparing a roofing material. The method includes (a) obtaining a coated substrate, (b) obtaining a plurality of roofing granules, wherein the plurality of roofing granules comprises from 50% to 100% of unitary, uncoated, non-mineral based particles, and (c) applying the plurality of roofing granules to a surface of the coated substrate to form a roofing material.

In an embodiment, the step of applying the plurality of roofing granules to the surface of the coated substrate is conducted to achieve an average surface coverage amount of the roofing granules of greater than 95%. In an embodiment, the step of applying the plurality of roofing granules to the surface of the coated substrate is conducted to achieve an average surface coverage amount of the roofing granules of greater than 90%. In an embodiment, the step of applying the plurality of roofing granules to the surface of the coated substrate is conducted to achieve an average surface coverage amount of the roofing granules of greater than 85%. In an embodiment, the step of applying the plurality of roofing granules to the surface of the coated substrate is conducted to achieve an average surface coverage amount of the roofing granules of greater than 80%. In an embodiment, the step of applying the plurality of roofing granules to the surface of the coated substrate is conducted to achieve an average surface coverage amount of the roofing granules of greater than 75%. In an embodiment, the step of applying the plurality of roofing granules to the surface of the coated

## 11

substrate is conducted to achieve an average surface coverage amount of the roofing granules of greater than 70%. In an embodiment, the step of applying the plurality of roofing granules to the surface of the coated substrate is conducted to achieve an average surface coverage amount of the roofing granules of greater than 65%. In an embodiment, the step of applying the plurality of roofing granules to the surface of the coated substrate is conducted to achieve an average surface coverage amount of the roofing granules of greater than 60%. In an embodiment, the step of applying the plurality of roofing granules to the surface of the coated substrate is conducted to achieve an average surface coverage amount of the roofing granules of greater than 55%. In an embodiment, the step of applying the plurality of roofing granules to the surface of the coated substrate is conducted to achieve an average surface coverage amount of the roofing granules of greater than 50%.

In an embodiment, asphaltic shingles with reduced weight can be obtained by using non-mineral based roofing granules according to embodiments of the disclosure as the surfacing media to reduce the weight of the shingle. Typically, mineral-based roofing granules have a density in a range exceeding 2.5 g/cm<sup>3</sup> and constitute a significant part of the total shingle weight. According to embodiments of this disclosure, by using non-mineral based roofing granules as the surfacing media, the weight of the shingles can be reduced. The shingle(s) with lighter weight can have benefits of being easier to handle and install, easier to carry to the job site, and lowered transportation cost.

According to an embodiment, the non-mineral based roofing granules or particles have a high UV opacity to protect the asphaltic coating of the substrate underneath, and have the durability for long term outdoor exposure required for roofing applications.

According to an embodiment, the non-mineral based roofing granules or particles can be applied to molten asphalt in a moving web via gravity feed, or another system, including, e.g., a high speed granule system which does not rely on gravity to apply the granules during a shingle manufacturing process to obtain shingles with a lighter weight. According to another embodiment, the non-mineral based roofing granules or particles can be applied to the molten asphalt surface via equipment that is designed to apply particles onto a moving web in a precise manner, such as, e.g., a high-speed particle applicator, electrostatic deposition, particle spraying, and combinations thereof. According to an embodiment, the non-mineral based roofing granules or particles can be applied throughout the entire shingle surface or in certain areas, such as in the upper exposure area, to form the shingles with desirable properties while reducing the potential cost impact. According to an embodiment, the non-mineral based roofing granules or particles can be applied to the back of the shingles to increase the shingle thickness, while keeping the weight of the shingle lowered. According to another embodiment, the non-mineral based roofing granules or particles may be combined with mineral-based roofing granules to form blends that may deliver unique textures and/or aesthetics on the shingle surface.

According to an embodiment, the synthetic or non-mineral based roofing granules with increased solar reflectance can be obtained by using non-mineral based particles having suitable sizes and geometries that can result in a high surface coverage over an asphaltic shingle surface. According to another embodiment, the non-mineral based roofing gran-

## 12

ules or particles can contain solar reflective pigments and/or additives to provide high solar reflectivity while maintaining desirable aesthetics.

In another embodiment, roofing materials, e.g., shingles, with improved staining resistance can be obtained by applying the non-mineral based roofing granules in the exposure area or the upper surface of the shingles. The improved staining resistance can be achieved by using non-mineral based granules or particles that have much less surface porosity and/or lower surface energy or lower affinity to prevent the spreading of oils migrating from the asphaltic substrates. Mineral-based roofing granules may have rough surfaces and surface porosity from crushing of the mineral rock base that can readily absorb asphaltic oils. In addition, the mineral surfaces may have very high surface energy, such that the asphaltic oils will be absorbed to lower the surface energy, which thereby results in staining. To reduce these effects and the staining, mineral-based roofing granules may be treated with silicate coatings to seal off the surface porosity and to lower the surface energetics for reducing its staining potential. By using the non-mineral based granules or particles according to embodiments of this disclosure, the staining potential can be reduced by such granules or particles that contain low surface porosity and/or low surface energy without additional surface treatments. In addition, mineral-based roofing granules may be blended with mineral oils or slate oils to help reduce the dust formation during transportation, which can lead to color change as the shingles made with such granules are weathered outdoors. However, by using the non-mineral based granules or particles according to embodiments of this disclosure as the roofing surfacers, there is no need to apply mineral oils or slate oils as dust controlling agents.

In another embodiment, roofing materials (e.g., shingles) with improved color saturations or improved gloss appearance can be obtained by using the non-mineral based granules on the outer surface or the exposure areas. Typical mineral-based roofing granules are coated with pigmented metal-silicate coatings that inefficiently cover the mineral surfaces, which result in granule colors that are far from the saturated color space. Also, the mineral surfaces are relatively rough due to crevices and/or pores that are formed from crushing and fracturing during the granule making process, which can lead to dull surfaces with relatively low gloss surface characteristics. This is especially visible along the cut edge of shingles where the granule coatings were crushed by the cutting knife to result in an “edge line” of granule showing its base mineral color. However, by using the non-mineral based granules or particles according to embodiments of this disclosure as the surfacing media, the color can be more evenly provided throughout the particles for reaching the saturated color and the color will be maintained even if the particles are severed. Also, according to an embodiment, the surface of the non-mineral based particles can have a high gloss for achieving desirable aesthetics in matching other roofing elements having high gloss surfaces.

According to one embodiment, the particles can have a greater affinity to the substrate materials or coatings, such that the particles will have low rub loss and/or reduced granule loss over time.

According to an embodiment, the particles can be transported or processed during a typical shingle making process without generating air-borne dust, as in the case of mineral-based roofing granules, such that the measure for dust control or additional dust handling steps can be reduced or eliminated.

According to an embodiment, the particles can improve the impact resistance of the shingle and/or membranes by absorbing the impact energy via plasticity or viscoelastic properties of the polymeric materials, or via a collapsible structural of the particles, including, e.g., a core/shell construction.

According to another embodiment, the particles can have a surface texture to enhance the aesthetics of the finished roof surfaces and/or surface treatments to enhance adhesions to substrates.

According to an embodiment, the non-mineral based particles or granules and/or a roofing material prepared from such non-mineral based particles or granules can exhibit improved algae resistance as compared to, e.g., mineral based particles or granules and/or a roofing material prepared with mineral based particles or granules.

### EXAMPLES

Specific embodiments of the invention will now be demonstrated by reference to the following examples. It should be understood that these examples are disclosed by way of illustrating the invention and should not be taken in any way to limit the scope of the present invention.

#### Example 1

Samples of synthetic, non-mineral based particles suitable for outdoor exposures were obtained from a commercially available source and were compared to existing mineral-based roofing granules used for roofing shingles. Their colors were measured using a colorimeter (HunterLab XE colorimeter using D65 illumination and 10° observer) and are listed in the Table shown in FIG. 2 for direct comparison. Also, their total solar reflectance (TSR) was measured following ASTM C1549 using a D&S solar reflectometer (1.5 air mass). (See measured TSR data values shown in the Table of FIG. 2.)

The data shows that the non-mineral based particles can have a similar color space with an increased solar reflectance. For example, as shown in the data of the Table of FIG. 2, the mineral-based granule entitled "Light Black" has a 0.1 TSR, whereas the closely matched color of the non-mineral based granule entitled "DARK GRAY" has a 0.2 TSR. Also, as shown by the data for this Example, the non-mineral based particles can result in a higher color strength or a higher color saturation. (See, e.g., the E\* value in the data of the Table of FIG. 2, which is a measure of the color space from the center of the color sphere where the outer surface represents the most saturated color.) For example, as shown in the data of the Table of FIG. 2, the highest E\* value achieved by the mineral based granules was about 77 (see, e.g., mineral-based granules entitled "White"), whereas the highest E\* value achieved by the non-mineral based particles was greater than 95 (see, e.g., synthetic granules entitled "White 299").

#### Example 2

Asphaltic shingle samples covered by either mineral-based granules or non-mineral based granules were made and compared in the following manner. Approximately 200 grams of mineral based granules were obtained and applied onto a 4"×4" asphalt substrate by gravity feed to fully cover the entire surface of the substrate, followed by pressing using a 25-lb roller having diameter of 6". After the pressing, excessive granules were removed to form the shingle

surface. The same procedure was repeated for the non-mineral based granules to obtain shingle samples. Three granule colors were selected in each granule category (i.e., mineral-based granules and non-mineral based granules) (see, e.g., FIG. 3) and were made into the shingle form of a 4"×4" size as described above. The resultant shingle samples had a uniform granulated surface. The color of each of the prepared shingle samples, as well as their TSR values were measured. These measured values are shown in the Table of FIG. 4.

As can be seen by the data in the Table shown in FIG. 4, the shingle samples prepared with non-mineral based granules were found to have a lower weight per thickness per area as compared to the shingle samples prepared with mineral-based particles. For example, the mineral-based granulated shingle samples had a weight per thickness per area ranging from about 2.3 g/mil/ft<sup>2</sup> to about 2.6 g/mil/ft<sup>2</sup>, whereas the non-mineral based granulated shingle samples had a weight per thickness per area range of only about 1.5 g/mil/ft<sup>2</sup> to 1.9 g/mil/ft<sup>2</sup>. Thus, this example illustrates that shingle samples prepared with non-mineral based granules result in much less weight per roofing square, or thicker shingles at the same weight. The data also shows that the shingle samples made with non-mineral based granules have significantly higher TSR values, as compared to those made with mineral-based granules. (See, e.g., TSR values shown in the Table of FIG. 4.)

#### Example 3

Shingle samples were made using the same procedure as described in Example 2 above to test their staining resistance. For the mineral-based roofing granules, the roofing granule entitled "I-760" was selected in "white color". For the non-mineral based granules, the roofing granule entitled "RV Grey" was selected. The non-mineral based granules ("RV Grey") were also selected in the white color space and used for comparing with the selected mineral-based roofing granules ("I-760"). The prepared shingle samples were then tested for their staining resistance by placing the samples in a forced-air oven at 175° F. for 24 hours. The samples' color before and after the staining test were measured. The results are shown in the Table of FIG. 5 and also shown in FIG. 6 for visual comparison.

As can be seen from the data in the Table of FIG. 5, as well as the visual results of FIG. 6, the shingle sample prepared with mineral-based granules showed a significant darkening effect with a Delta E value of 3.3 due to the staining from the asphaltic substrate, whereas the shingle sample prepared with non-mineral based granules was not affected by asphalt staining and had a minimum change in color with a Delta E value of 0.4. These results can also be seen in FIG. 6, where the color of the shingle sample prepared with mineral-based particles is significantly changed after the staining test, which is undesirable from an aesthetic point of view, as compared to the color of the shingle sample prepared with non-mineral based particles.

Although the invention has been described in certain specific exemplary embodiments, many additional modifications and variations would be apparent to those skilled in the art in light of this disclosure. It is, therefore, to be understood that this invention may be practiced otherwise than as specifically described. Thus, the exemplary embodiments of the invention should be considered in all respects to be illustrative and not restrictive, and the scope of the

15

invention to be determined by any claims supportable by this application and the equivalents thereof, rather than by the foregoing description.

We claim:

1. A roofing material comprising:  
a coated substrate having (i) a top surface, (ii) a back surface, (iii) an upper portion comprising a headlap portion, and (iv) a lower portion comprising a buttlap portion, wherein the buttlap portion includes a plurality of tabs;

a backer strip attached to the back surface of the coated substrate, wherein the backer strip has (i) a top surface and (ii) a back surface; and

a plurality of roofing granules applied to (i) the plurality of tabs of the buttlap portion of the coated substrate, and (ii) at least a portion of the top surface of the backer strip,

wherein the plurality of roofing granules comprises from 50% to 100% of unitary, uncoated, non-mineral based particles, the non-mineral based particles comprising at least one of a thermoplastic polymer, filled polymers, filled rubbers, filled plastics, a polymer-sand composite, a rubber particle, a wood filled polymer, a bio-based particle, a thermoset material, a fiber-reinforced polymer, and combinations thereof,

wherein the plurality of roofing granules are applied at an average surface coverage amount of the roofing granules of greater than 55%, with the plurality of roofing granules being exposed across (i) the plurality of tabs of the buttlap portion of the coated substrate, and (ii) the at least a portion of the top surface of the backer strip,

wherein the roofing material is configured to be installed on a roof to form a roofing system, and

wherein, when the roofing material is installed on the roof to form the roofing system, the plurality of roofing granules forms an exposed surface of the roofing system.

2. The roofing material according to claim 1, wherein the substrate comprises one of a fiberglass mat, a polyester mat, a scrim, a coated scrim, or a combination thereof.

3. The roofing material according to claim 1, wherein the roofing material is one of a roofing shingle and a roofing tile.

4. The roofing material according to claim 1, wherein the roofing material is one of (i) an asphaltic shingle, (ii) a non-asphaltic shingle, and (ii) a polymer-modified asphalt shingle.

5. The roofing material according to claim 1, wherein each roofing granule of the plurality of roofing granules has a density of 1.2 g/cm<sup>3</sup> to 2.5 g/cm<sup>3</sup>.

6. The roofing material according to claim 1, wherein the non-mineral based particles comprise a synthetic particle.

7. The roofing material according to claim 1, wherein the non-mineral based particles comprise a thermoplastic polymer.

8. The roofing material according to claim 1, wherein the non-mineral based particles comprise filled polymers.

9. The roofing material according to claim 1, wherein the non-mineral based particles comprise filled rubbers.

10. The roofing material according to claim 1, wherein the non-mineral based particles comprise filled plastics.

11. The roofing material according to claim 1, wherein the non-mineral based particles comprise a polymer-sand composite.

12. The roofing material according to claim 1, wherein the non-mineral based particles comprise rubber particles.

16

13. The roofing material according to claim 1, wherein the non-mineral based particles comprise a wood filled polymer.

14. The roofing material according to claim 1, wherein the non-mineral based particles comprise bio-based particles.

15. The roofing material according to claim 1, wherein the non-mineral based particles comprise a thermoset material.

16. The roofing material according to claim 1, wherein the non-mineral based particles comprise a fiber-reinforced polymer.

17. The roofing material according to claim 1, wherein the at least one of a thermoplastic polymer, filled polymers, filled rubbers, filled plastics, a polymer-sand composite, a rubber particle, a wood filled polymer, a bio-based particle, a thermoset material, a fiber-reinforced polymer, and combinations thereof comprises a recycled material.

18. The roofing material according to claim 1, wherein the non-mineral based particles have an aspect ratio of from 1.5 to 50.

19. The roofing material according to claim 1, wherein the non-mineral based particles have a particle size of from #8 US mesh to #60 US mesh.

20. The roofing material according to claim 1, wherein less than 1% by weight of the plurality of roofing granules have a particle size of greater than #100 US mesh.

21. The roofing material according to claim 1, wherein the roofing material exhibits a lower weight per thickness as compared to a roofing material prepared with roofing granules comprising mineral based particles.

22. The roofing material according to claim 1, wherein the roofing material exhibits a weight per thickness of from 0.17 to 0.21 g/mil.

23. The roofing material according to claim 1, wherein the roofing material exhibits an improved staining resistance as compared to a roofing material prepared with roofing granules comprising mineral based particles.

24. The roofing material according to claim 1, wherein the roofing granules exhibit a total solar reflectance (TSR) of from 0.2 to 0.8 according to ASTM C1549.

25. The roofing material according to claim 1, wherein the roofing granules exhibit a higher color saturation as compared to roofing granules comprising mineral based particles.

26. A method of applying roofing granules to a roofing material, the method comprising:

obtaining a roofing material comprising:

(a) a coated substrate having (i) a top surface, (ii) a back surface, (iii) an upper portion comprising a headlap portion, and (iv) a lower portion comprising a buttlap portion, wherein the buttlap portion includes a plurality of tabs; and

(b) a backer strip attached to the back surface of the coated substrate, wherein the backer strip has (i) a top surface and (ii) a back surface;

obtaining a plurality of roofing granules, wherein the plurality of roofing granules comprises from 50% to 100% of unitary, uncoated, non-mineral based particles, the non-mineral based particles comprising at least one of a thermoplastic polymer, filled polymers, filled rubbers, filled plastics, a polymer-sand composite, a rubber particle, a wood filled polymer, a bio-based particle, a thermoset material, a fiber-reinforced polymer, and combinations thereof;

applying the plurality of roofing granules to the (i) the plurality of tabs of the buttlap portion of the coated substrate, and (ii) at least a portion of the top surface of the backer strip,

60  
65  
66  
67  
68  
69  
70  
71  
72  
73  
74  
75  
76  
77  
78  
79  
80  
81  
82  
83  
84  
85  
86  
87  
88  
89  
90  
91  
92  
93  
94  
95  
96  
97  
98  
99  
100  
101  
102  
103  
104  
105  
106  
107  
108  
109  
110  
111  
112  
113  
114  
115  
116  
117  
118  
119  
120  
121  
122  
123  
124  
125  
126  
127  
128  
129  
130  
131  
132  
133  
134  
135  
136  
137  
138  
139  
140  
141  
142  
143  
144  
145  
146  
147  
148  
149  
150  
151  
152  
153  
154  
155  
156  
157  
158  
159  
160  
161  
162  
163  
164  
165  
166  
167  
168  
169  
170  
171  
172  
173  
174  
175  
176  
177  
178  
179  
180  
181  
182  
183  
184  
185  
186  
187  
188  
189  
190  
191  
192  
193  
194  
195  
196  
197  
198  
199  
200  
201  
202  
203  
204  
205  
206  
207  
208  
209  
210  
211  
212  
213  
214  
215  
216  
217  
218  
219  
220  
221  
222  
223  
224  
225  
226  
227  
228  
229  
230  
231  
232  
233  
234  
235  
236  
237  
238  
239  
240  
241  
242  
243  
244  
245  
246  
247  
248  
249  
250  
251  
252  
253  
254  
255  
256  
257  
258  
259  
2510  
2511  
2512  
2513  
2514  
2515  
2516  
2517  
2518  
2519  
2520  
2521  
2522  
2523  
2524  
2525  
2526  
2527  
2528  
2529  
2530  
2531  
2532  
2533  
2534  
2535  
2536  
2537  
2538  
2539  
2540  
2541  
2542  
2543  
2544  
2545  
2546  
2547  
2548  
2549  
2550  
2551  
2552  
2553  
2554  
2555  
2556  
2557  
2558  
2559  
2560  
2561  
2562  
2563  
2564  
2565  
2566  
2567  
2568  
2569  
2570  
2571  
2572  
2573  
2574  
2575  
2576  
2577  
2578  
2579  
2580  
2581  
2582  
2583  
2584  
2585  
2586  
2587  
2588  
2589  
2590  
2591  
2592  
2593  
2594  
2595  
2596  
2597  
2598  
2599  
25100  
25101  
25102  
25103  
25104  
25105  
25106  
25107  
25108  
25109  
25110  
25111  
25112  
25113  
25114  
25115  
25116  
25117  
25118  
25119  
25120  
25121  
25122  
25123  
25124  
25125  
25126  
25127  
25128  
25129  
25130  
25131  
25132  
25133  
25134  
25135  
25136  
25137  
25138  
25139  
25140  
25141  
25142  
25143  
25144  
25145  
25146  
25147  
25148  
25149  
25150  
25151  
25152  
25153  
25154  
25155  
25156  
25157  
25158  
25159  
25160  
25161  
25162  
25163  
25164  
25165  
25166  
25167  
25168  
25169  
25170  
25171  
25172  
25173  
25174  
25175  
25176  
25177  
25178  
25179  
25180  
25181  
25182  
25183  
25184  
25185  
25186  
25187  
25188  
25189  
25190  
25191  
25192  
25193  
25194  
25195  
25196  
25197  
25198  
25199  
25200  
25201  
25202  
25203  
25204  
25205  
25206  
25207  
25208  
25209  
25210  
25211  
25212  
25213  
25214  
25215  
25216  
25217  
25218  
25219  
25220  
25221  
25222  
25223  
25224  
25225  
25226  
25227  
25228  
25229  
25230  
25231  
25232  
25233  
25234  
25235  
25236  
25237  
25238  
25239  
25240  
25241  
25242  
25243  
25244  
25245  
25246  
25247  
25248  
25249  
25250  
25251  
25252  
25253  
25254  
25255  
25256  
25257  
25258  
25259  
25260  
25261  
25262  
25263  
25264  
25265  
25266  
25267  
25268  
25269  
25270  
25271  
25272  
25273  
25274  
25275  
25276  
25277  
25278  
25279  
25280  
25281  
25282  
25283  
25284  
25285  
25286  
25287  
25288  
25289  
25290  
25291  
25292  
25293  
25294  
25295  
25296  
25297  
25298  
25299  
25300  
25301  
25302  
25303  
25304  
25305  
25306  
25307  
25308  
25309  
25310  
25311  
25312  
25313  
25314  
25315  
25316  
25317  
25318  
25319  
25320  
25321  
25322  
25323  
25324  
25325  
25326  
25327  
25328  
25329  
25330  
25331  
25332  
25333  
25334  
25335  
25336  
25337  
25338  
25339  
25340  
25341  
25342  
25343  
25344  
25345  
25346  
25347  
25348  
25349  
25350  
25351  
25352  
25353  
25354  
25355  
25356  
25357  
25358  
25359  
25360  
25361  
25362  
25363  
25364  
25365  
25366  
25367  
25368  
25369  
25370  
25371  
25372  
25373  
25374  
25375  
25376  
25377  
25378  
25379  
25380  
25381  
25382  
25383  
25384  
25385  
25386  
25387  
25388  
25389  
25390  
25391  
25392  
25393  
25394  
25395  
25396  
25397  
25398  
25399  
25400  
25401  
25402  
25403  
25404  
25405  
25406  
25407  
25408  
25409  
25410  
25411  
25412  
25413  
25414  
25415  
25416  
25417  
25418  
25419  
25420  
25421  
25422  
25423  
25424  
25425  
25426  
25427  
25428  
25429  
25430  
25431  
25432  
25433  
25434  
25435  
25436  
25437  
25438  
25439  
25440  
25441  
25442  
25443  
25444  
25445  
25446  
25447  
25448  
25449  
25450  
25451  
25452  
25453  
25454  
25455  
25456  
25457  
25458  
25459  
25460  
25461  
25462  
25463  
25464  
25465  
25466  
25467  
25468  
25469  
25470  
25471  
25472  
25473  
25474  
25475  
25476  
25477  
25478  
25479  
25480  
25481  
25482  
25483  
25484  
25485  
25486  
25487  
25488  
25489  
25490  
25491  
25492  
25493  
25494  
25495  
25496  
25497  
25498  
25499  
25500  
25501  
25502  
25503  
25504  
25505  
25506  
25507  
25508  
25509  
25510  
25511  
25512  
25513  
25514  
25515  
25516  
25517  
25518  
25519  
25520  
25521  
25522  
25523  
25524  
25525  
25526  
25527  
25528  
25529  
25530  
25531  
25532  
25533  
25534  
25535  
25536  
25537  
25538  
25539  
25540  
25541  
25542  
25543  
25544  
25545  
25546  
25547  
25548  
25549  
25550  
25551  
25552  
25553  
25554  
25555  
25556  
25557  
25558  
25559  
25560  
25561  
25562  
25563  
25564  
25565  
25566  
25567  
25568  
25569  
25570  
25571  
25572  
25573  
25574  
25575  
25576  
25577  
25578  
25579  
25580  
25581  
25582  
25583  
25584  
25585  
25586  
25587  
25588  
25589  
25590  
25591  
25592  
25593  
25594  
25595  
25596  
25597  
25598  
25599  
25600  
25601  
25602  
25603  
25604  
25605  
25606  
25607  
25608  
25609  
25610  
25611  
25612  
25613  
25614  
25615  
25616  
25617  
25618  
25619  
25620  
25621  
25622  
25623  
25624  
25625  
25626  
25627  
25628  
25629  
25630  
25631  
25632  
25633  
25634  
25635  
25636  
25637  
25638  
25639  
25640  
25641  
25642  
25643  
25644  
25645  
25646  
25647  
25648  
25649  
25650  
25651  
25652  
25653  
25654  
25655  
25656  
25657  
25658  
25659  
25660  
25661  
25662  
25663  
25664  
25665  
25666  
25667  
25668  
25669  
25670  
25671  
25672  
25673  
25674  
25675  
25676  
25677  
25678  
25679  
25680  
25681  
25682  
25683  
25684  
25685  
25686  
25687  
25688  
25689  
25690  
25691  
25692  
25693  
25694  
25695  
25696  
25697  
25698  
25699  
25700  
25701  
25702  
25703  
25704  
25705  
25706  
25707  
25708  
25709  
25710  
25711  
25712  
25713  
25714  
25715  
25716  
25717  
25718  
25719  
25720  
25721  
25722  
25723  
25724  
25725  
25726  
25727  
25728  
25729  
25730  
25731  
25732  
25733  
25734  
25735  
25736  
25737  
25738  
25739  
25740  
25741  
25742  
25743  
25744  
25745  
25746  
25747  
25748  
25749  
25750  
25751  
25752  
25753  
25754  
25755  
25756  
25757  
25758  
25759  
25760  
25761  
25762  
25763  
25764  
25765  
25766  
25767  
25768  
25769  
25770  
25771  
25772  
25773  
25774  
25775  
25776  
25777  
25778  
25779  
25780  
25781  
25782  
25783  
25784  
25785  
25786  
25787  
25788  
25789  
25790  
25791  
25792  
25793  
25794  
25795  
25796  
25797  
25798  
25799  
25800  
25801  
25802  
25803  
25804  
25805  
25806  
25807  
25808  
25809  
25810  
25811  
25812  
25813  
25814  
25815  
25816  
25817  
25818  
25819  
25820  
25821  
25822  
25823  
25824  
25825  
25826  
25827  
25828  
25829  
25830  
25831  
25832  
25833  
25834  
25835  
25836  
25837  
25838  
25839  
25840  
25841  
25842  
25843  
25844  
25845  
25846  
25847  
25848  
25849  
25850  
25851  
25852  
25853  
25854  
25855  
25856  
25857  
25858  
25859  
25860  
25861  
25862  
25863  
25864  
25865  
25866  
25867  
25868  
25869  
25870  
25871  
25872  
25873  
25874  
25875  
25876  
25877  
25878  
25879  
25880  
25881  
25882  
25883  
25884  
25885  
25886  
25887  
25888  
25889  
25890  
25891  
25892  
25893  
25894  
25895  
25896  
25897  
25898  
25899  
25900  
25901  
25902  
25903  
25904  
25905  
25906  
25907  
25908  
25909  
25910  
25911  
25912  
25913  
25914  
25915  
25916  
25917  
25918  
25919  
25920  
25921  
25922  
25923  
25924  
25925  
25926  
25927  
25928  
25929  
25930  
25931  
25932  
25933  
25934  
25935  
25936  
25937  
25938  
25939  
25940  
25941  
25942  
25943  
25944  
25945  
25946  
25947  
25948  
25949  
25950  
25951  
25952  
25953  
25954  
25955  
25956  
25957  
25958  
25959  
25960  
25961  
25962  
25963  
25964  
25965  
25966  
25967  
25968  
25969  
25970  
25971  
25972  
25973  
25974  
25975  
25976  
25977  
25978  
25979  
25980  
25981  
25982  
25983  
25984  
25985  
25986  
25987  
25988  
25989  
25990  
25991  
25992  
25993  
25994  
25995  
25996  
25997  
25998  
25999  
25100  
25101  
25102  
25103  
25104  
25105  
25106  
25107  
25108  
25109  
25110  
25111  
25112  
25113  
25114  
25115  
25116  
25117  
25118  
25119  
25120  
25121  
25122  
25123  
25124  
25125  
25126  
25127  
25128  
25129  
25130  
25131  
25132  
25133  
25134  
25135  
25136  
25137  
25138  
25139  
25140  
25141  
25142  
25143  
25144  
25145  
25146  
25147  
25148  
25149  
25150  
25151  
25152  
25153  
25154  
25155  
25156  
25157  
25158  
25159  
25160  
25161  
25162  
25163  
25164  
25165  
25166  
25167  
25168  
25169  
25170  
25171  
25172  
25173  
25174  
25175  
25176  
25177  
25178  
25179  
25180  
25181  
25182  
25183  
25184  
25185  
25186  
25187  
25188  
25189  
25190  
25191  
25192  
25193  
25194  
25195  
25196  
25197  
25198  
25199<br

wherein the applying the plurality of roofing granules is conducted to achieve an average surface coverage amount of the roofing granules of greater than 55%, with the plurality of roofing granules being exposed across (i) the plurality of tabs of the buttlap portion of 5 the coated substrate, and (ii) the at least a portion of the top surface of the backer strip,  
wherein the roofing material is configured to be installed on a roof to form a roofing system, and  
wherein, when the roofing material is installed on the roof 10 to form the roofing system, the plurality of roofing granules forms an exposed surface of the roofing system.

**27.** The method according to claim 26, wherein the substrate comprises one of a fiberglass mat, a polyester mat, 15 a scrim, a coated scrim, or a combination thereof.

**28.** The method according to claim 26, wherein each roofing granule of the plurality of roofing granules has a density of 1.2 g/cm<sup>3</sup> to 2.5 g/cm<sup>3</sup>.

**29.** The method according to claim 26, wherein the 20 non-mineral based particles comprise a synthetic particle.

**30.** The method according to claim 26, wherein the at least one of a thermoplastic polymer, filled polymers, filled rubbers, filled plastics, a polymer-sand composite, a rubber particle, a wood filled polymer, a bio-based particle, a 25 thermoset material, a fiber-reinforced polymer, and combinations thereof comprises a recycled material.

\* \* \* \* \*